

[54] **METHOD CONCENTRATE AND SOLUTION FOR SIMULTANEOUS CLEANING, DEGREASING AND REMOVAL OF THE LUBRICANT CARRIER LAYER FROM IRON AND STEEL WORKPIECES**

[75] Inventor: **Peter Jorns**, Frankfurt am Main, Germany

[73] Assignee: **Oxy Metal Industries Corporation**, Warren, Mich.

[22] Filed: **Feb. 13, 1973**

[21] Appl. No.: **332,055**

[30] **Foreign Application Priority Data**

Feb. 19, 1972 Germany ..... 2207848

[52] U.S. Cl. ..... **134/2; 134/40; 252/156; 252/387**

[51] Int. Cl. ..... **C23g 1/16; C11d 7/16; C23g 1/20**

[58] **Field of Search** ..... 252/146, 147, 387, 79.1, 252/139, 156, 158, 173, 389 R; 134/40, 41, 2

[56]

**References Cited**

**UNITED STATES PATENTS**

|           |         |                  |          |
|-----------|---------|------------------|----------|
| 2,499,261 | 2/1950  | Rosenbloom ..... | 117/127  |
| 2,813,075 | 11/1957 | Brooke .....     | 252/8.55 |
| 2,916,459 | 12/1959 | Arnold .....     | 252/152  |
| 3,015,630 | 1/1962  | Thompson .....   | 252/101  |
| 3,151,087 | 9/1964  | Ryznar .....     | 252/387  |
| 3,668,132 | 6/1972  | Finder .....     | 134/2    |
| 3,723,334 | 3/1973  | Maurer .....     | 21/2.7 R |

*Primary Examiner*—Barry S. Richman

*Assistant Examiner*—Dale Lovercheck

*Attorney, Agent, or Firm*—Arthur E. Kluegel; Richard P. Mueller; B. F. Claeboe

[57]

**ABSTRACT**

Alkaline concentrate and aqueous solution for removing lubricant carrier and residue from iron containing surfaces. The alkaline solution contains phosphate ions and either cobalt or nickel ions or a mixture of the two. Use of the solution helps prevent inter stage rusting and the problems resulting therefrom.

**4 Claims, No Drawings**

**METHOD CONCENTRATE AND SOLUTION FOR SIMULTANEOUS CLEANING, DEGREASING AND REMOVAL OF THE LUBRICANT CARRIER LAYER FROM IRON AND STEEL WORKPIECES**

**BACKGROUND OF THE INVENTION**

Prior to the forming of metal workpieces, it is customary to apply chemical coatings, particularly phosphate layers, to their surfaces, and to carry out the forming in the presence of lubricants. The residues located on the surface after the forming may interfere with the further processing or use of the workpieces, so that their removal is necessary.

Aqueous alkaline solutions based on soluble phosphates are often used for simultaneous removal (cleaning) of the lubricant carrier layers and the lubricant residues. Salts of orthophosphoric acid and/or salts of condensed phosphates come into consideration as phosphates. However, it has been found that the treated workpieces are subject to considerable danger of rusting upon leaving the removal zone, and the rust occurs particularly in the transition zones between processing stages. The susceptibility to rust is also at least partially due to the deformation of the workpiece, and thus the change in the surface structure of the material. In automatically timed systems, long carry-over times can sometimes intervene between the cleaning bath and the rinsing baths. The parts cleaned with the phosphate solution rust slightly during this time. However, this is undesirable and greatly interferes with subsequent treatments, especially for subsequent phosphatation.

**THE INVENTION**

It has not been found that this disadvantageous susceptibility to rust can be avoided by adding to the cleaning solution soluble metal compounds of nickel and/or cobalt, preferably cobalt.

The rust-inhibiting effect is attained upon the addition of at least 0.05 g/l of the metal compound, calculated as cobalt and/or nickel. Quantities of more than 10 g/l offer no additional advantage. Preferably, 0.1 to 2 g/l of the metal or metals is added.

Suitable cobalt salts include cobalt nitrate, cobalt sulfate, cobalt acetate, cobalt chloride. Suitable nickel compounds include nickel nitrate, nickel sulfate, nickel chloride, nickel acetate.

The phosphates used in the cleaner in accordance with the invention primarily include those of condensed phosphoric acids, especially pyrophosphoric acid. The phosphate content advantageously amounts to 5 to 80 g/l, preferably 15 to 50 g/l, calculated as  $P_2O_5$ . The aqueous cleaning solution normally has a pH of 8-13, and preferably the pH is kept in the range of 9-12. In order to increase the cleansing effect of the aqueous solution, surface-active substances and/or solvents may be included. Suitable surfactants include anionic surfactants such as alkybenzenesulfonates, fatty alcohol sulfates, etc., or nonionic surfactants, such as ethylene oxide addition products to alkylphenols or fatty alcohols. When nonionic surfactants are used, it is necessary to make sure that these surfactants possess sufficient solubility at the concentration and temperature used. Preferably, anionic surfactants are used. It is advantageous to add 0.1-3 g/l wetting agent. Organic solvents, such as higher-boiling hydrocarbons (kero-

sene, petroleum), glycols, or polyglycols are advantageously used in quantities of 0.5-10 g/l.

The cleansing solution in accordance with the invention can advantageously be prepared from a solid cleanser concentrate. Such a concentrate preferably has the following composition:

|    |          |                           |
|----|----------|---------------------------|
| 10 | 70 - 90% | $Na_4P_2O_7$              |
|    | 0 - 10%  | $Na_5P_3O_{10}$           |
|    | 1 - 10%  | $Co(NO_3)_2 \cdot 6 H_2O$ |
|    | 0 - 5%   | surfactant                |
|    | 0 - 20%  | solvent                   |

The use of the cleanser in accordance with the invention will be explained in greater detail on the basis of the following examples:

**EXAMPLE I**

Intermediate stages from shock-absorber piping manufacture, which were covered with a residual phosphate and lubricant layer, were cleaned in a cleanser solution containing

|    |        |                                                 |
|----|--------|-------------------------------------------------|
| 25 | 46 g/l | $Na_4P_2O_7$ ; calc.                            |
|    | 2 g/l  | $Na_5P_3O_{10}$ ; calc.                         |
|    | 1 g/l  | polyethylene glycol (molecular weight ca. 4000) |

for 10 min. at 95°C. After this time, the phosphate and lubricant residues were completely removed from the surface of the workpiece. Following the cleaning, the parts were slowly introduced into a water rinsing bath within 60 sec, and rinsed vigorously there.

During the transport of the workpieces from the cleansing bath to the water rinsing bath, a very thick layer of rust was formed.

In a parallel experiment, 1.24 g/l  $Co(NO_3)_2 \cdot 6 H_2O$  (corresponding to 0.25 g/l Co) were added to the cleaning solution. In this experiment, no formation of heavy rust on the workpieces occurred.

During the subsequently performed phosphatation, when the Co-free cleaner bath was used, phosphate layers flecked irregularly with rust were formed, and led to substantial disturbances during the subsequent deformation stage. When the Co-containing cleaner bath was used, no difficulties of this type occurred in the phosphatation and shaping processes.

**EXAMPLE II**

In order to determine the influence of the Co concentration on the prevention of heavy rust formation, 0-5 g/l of Co in the form of cobalt nitrate were added to the cleaning bath according to Example I. In the various cleaning baths, drawing blanks covered with residual phosphate and lubricant layers were cleaned for 10 min at 95°C. The cleaned parts were then kept in the vapor atmosphere of the cleaning bath up to the beginning of heavy rust formation. The experimental results thus obtained are presented in the following table.

**TABLE**

|    | Addition, g/l Co | Beginning of heavy rust formation after ca.... minutes |
|----|------------------|--------------------------------------------------------|
| 65 | 0.               | 0.2                                                    |
|    | 0.02             | 0.2                                                    |
|    | 0.05             | 1                                                      |
|    | 0.1              | 3                                                      |
|    | 1.0              | 10                                                     |
|    | 2.0              | 15                                                     |

TABLE-continued

| Addition, g/l Co | Beginning of heavy rust formation<br>after ca.... minutes |
|------------------|-----------------------------------------------------------|
| 5.0              | 15                                                        |

## EXAMPLE III

Instead of cobalt nitrate, 0.25 g/l Ni as nickel sulfate was added to the cleaning bath according to Example I. In the cleaning of drawing blanks, no heavy rust formation was observed, even in the case of a prolonged waiting time between cleaning and rinsing bath.

What we claim is:

1. A method for the simultaneous cleaning, degreasing and removal of a cold-forming lubricant carrier layer from workpieces containing iron comprising con-

10 tacting said workpiece with an aqueous alkaline solution comprising 5-80 g/l phosphate ion and at least 0.05 g/l of a metal ion selected from the group consisting of cobalt, nickel and mixtures thereof, and having a pH adjusted to a value between 8 and 13 for at least one minute.

2. The method of claim 1 wherein said metal ion is present in a concentration of from 0.1 to 2.0 g/l.

3. An alkaline phosphate-containing aqueous solution for the simultaneous cleaning, degreasing and removal of a cold forming lubricant carrier layer from workpieces containing iron, comprising 5-80 g/l phosphate ion and at least 0.05 g/l of cobalt ion and having a pH adjusted to a value between 8 and 13.

15 4. The solution according to claim 3 wherein the cobalt ion is present in a concentration of about 0.1 to 2.0 g/l.

\* \* \* \* \*

20

25

30

35

40

45

50

55

60

65